

## UNITED STATES PATENT OFFICE

2,357,989

## SMOKELESS POWDER

Elton R. Allison, Washington, D. C., assignor to  
 Hercules Powder Company, Wilmington, Del.,  
 a corporation of Delaware

No Drawing. Application April 1, 1942,  
 Serial No. 437,229

6 Claims. (CL. 52—13)

This invention relates to an improved smokeless powder and to a method for its preparation. In more particular, the invention relates to an improved smokeless powder, especially adapted for firing at sub-zero temperatures and to a method of compounding such a powder.

In order to obtain progressive-burning smokeless powder, the art has developed various methods for surface-coating powder grains with a variety of materials. This surface coating so modifies the various powder grains that their burning characteristics may be controlled, i. e., as the powder burns from the surface inwardly, the successively exposed surfaces contain gradually less and less of the surface-coating material, and the combustion of the grains increases in speed as time of burning progresses.

Coatings of many different types have been used and each one has advantages which make powder so coated suitable for special purposes. Some disadvantages have been encountered with surface-coated powders due to fouling of the barrel, difficulties of ignition, high breech pressures when fired at low temperatures, clustering of the grains after coating, and the like, but for the most part, coated powder grains have been found very desirable.

It has been shown in the prior art that one of the most difficult problems facing the manufacturer of progressive-burning powder is the compounding of progressive-burning powder grains which will perform satisfactorily in rifles when they are shot at normal temperature, and also when they are shot at sub-zero temperature. The use of rifles at sub-zero temperature is becoming increasingly important because of aerial warfare. The temperatures experienced in aerial combat are usually well below zero, sometimes dropping as low as —40 or —50° F., and the performance of rifles, especially the rifles of the machine-gun type, is of extreme importance as a hangfire or an exceptionally high breech pressure may disrupt the workings of the gun to a point where the aircraft is forced out of battle.

The problem of controlling the operation of powders at sub-zero temperatures is shown by prior art Patent 2,159,208. Thus, improvements over normal powder may be obtained by colloidizing the nitrocellulose with anhydrous solvent alcohols instead of the normally water-containing solvents. The alcohol, in general use, contains usually about 5% water and produces a powder grain which has a decided tendency to cause high breech pressures, especially when the powder is of the double base type, i. e., containing in addition to nitrocellulose, a liquid explosive nitric ester such as nitroglycerin. The colloidizing of the powder with anhydrous solvents produces a grain structure which, upon firing at low temperature, gives improved results because the num-

ber of high breech pressure shots is materially reduced.

In addition to the use of anhydrous solvents, the control of high breech pressure shots obtained when firing a rifle at sub-zero temperature may be alleviated by the use of a particular coating method. Thus, for example, U. S. Patent 2,179,330, shows that a double base powder, when coated at a temperature below 55° C. with various deters, produces a finished powder that is characterized by a minimum number of high breech pressure shots.

Although the prior art has shown methods of reducing the number of high breech pressure shots obtained with various double base progressive-burning powders when they are fired at sub-zero temperature, the difficulties encountered due to hangfires, i. e., the delay of actual ignition of the powder and increased time that the bullet is in the barrel after the primer has been struck has not been adequately solved. The hangfire presents a very serious disadvantage, especially to the operation of rapid fire rifles, such as the automatic rifle and the machine gun, and it is absolutely necessary that a powder be produced which prevents hangfires when the powder is fired either at normal temperatures or at sub-zero temperatures. In addition to a powder which will not cause hangfires, the powder should also be characterized by a burning characteristic which will not tend to give excessively high breech pressures.

It is an object of this invention to produce a progressive-burning smokeless powder that is suitable for firing at sub-zero temperatures and which will not develop hangfires.

It is another object of this invention to produce a smokeless powder composition which is easily ignited, which burns at proper pressures to give desired ballistics and which may be used at normal or sub-normal temperatures without danger of hangfires or high breech pressures.

The objects of this invention have been accomplished by producing a smokeless powder composition which comprises an admixture of coated double base powder grains which, in themselves, will not produce excessively high breech pressures when fired at sub-zero temperatures and single base powder grains of approximately the same granulation as the said double base powder grains.

In more particular, the new and improved powder, in accordance with the present invention, is manufactured by mechanically admixing powder grains of the double base and single base types together. The double base component provides the necessary power, furnishes the ballistics desired in regard to velocity, and maintains the breech pressure within ranges which will not be harmful to the rifle barrel, while the single base powder component provides the necessary ease of

ignition and insures against hangfires. The admixture need only contain a minor amount of single base powder, but this single base powder must be of a granulation which will not segregate after being evenly distributed throughout the double base powder grains. In order to accomplish this desirable intimate admixing, it has been found that grains of substantially the same granulation and substantially the same specific gravity give the best results.

The admixtures which have been found very useful for controlling breech pressures and hangfires are admixtures of coated double base smokeless powders and single base smokeless powders in which the single base component is present within the range of between about 10% and about 30%. Reduction of the single base component below about 10% tends to cause hangfires, while increasing the percentage above about 30% prevents the ballistic advantages inherent within double base powders from exerting their true influence.

The double base powder grains which have been found most useful for admixture with single base grains in accordance with this invention are any powder grains which have been manufactured in a manner that provides ballistics which will not increase breech pressures when fired at sub-zero temperatures such as, for example, as disclosed by U. S. 2,159,208 and 2,179,330. It was found that the preferable means of producing such a powder is to provide a base grained double base smokeless powder and surface modify this base grain with an admixture of a non-volatile, non-explosive organic material which is a non-solvent for the nitrocellulose but which is compatible therewith, and a solvent for the said nitrocellulose. The coating procedure is carried out at a temperature less than about 55° C. as temperatures higher than about 55° C. will produce a coated powder which, if shot after sub-zero temperatures, will produce high breech pressures.

Examples of the deterrent which may be utilized to coat the grains of the double base smokeless powder at below 55° C. and in conjunction with a solvent for the nitrocellulose may be, for example, the alkyl esters of the fatty acids, terpene phthalates, rosin esters, synthetic lacquer resins as the modified or unmodified polyhydric alcohol-polybasic acid resins, rosins, hydrogenated rosins, and the like.

The solvents which may be used for assisting in the coating of the double base smokeless powder grains with the above-described deterrents are, for example, ethyl acetate, butyl acetate, mixtures of alcohol and ether and any other solvents for nitrocellulose which have a boiling point of from about 35° C. to about 180° C., and preferably from about 70° C. to about 130° C., or such non-volatile solvents as the alkyl phthalates. The process of producing such surface-modified double base powder grains is more fully described in U. S. Patent 2,179,330.

The single base powder grains which may be used for the present invention are prepared in the normal accepted manner, i. e., the nitrocellulose is colloided with solvents such as ether-alcohol, extruded through dies and granulated to the desired grain size. Thereafter, the solvent is recovered and the powder water dried, air dried, glazed, and sieved.

A desirable single base powder grain for use in accordance with this invention may be produced by colloiding 100 pounds of nitrocellulose having a nitrogen content of about 13% and con-

taining about 1% by weight diphenylamine with 100 pounds of an ether-alcohol admixture in a W and P mixer, extruding the colloided material through a press and granulating the strands produced into the desired grain size, after which the normal solvent recovery, water-dry, air-dry, glazing and sieving operations are carried out.

Now having described the manufacture of the double base powder grains and the single base powder grains which may be used as components of powder produced in accordance with this invention, there follows a description of tests of various powders and admixtures which illustrate by comparison the invention and conclusively show the nature of the improvements obtained.

#### COMPARISON I

In this comparison the improvement obtained by using a blend of powders in accordance with this invention regarding hangfires is shown.

#### Example A

A double base powder containing 20% nitroglycerin and granulated .045-.015 x 1/11 was coated with 1.25% rosin and 1.5% DNT and then fired at 77° F. and -50° F. The results of pressure and barrel time from firing 10 rounds in a .25/35 W. C. F. rifle with a 23 grain charge were:

| Temp.   | Pressure |        |        | Barrel time, sec./1,000 |      |       |
|---------|----------|--------|--------|-------------------------|------|-------|
|         | Min.     | Mean   | Max.   | Min.                    | Mean | Max.  |
| 77° F.  | 31,100   | 33,900 | 36,400 | 2.44                    | 2.89 | 3.96  |
| -50° F. | 22,600   | 28,400 | 31,000 | 2.80                    | 4.27 | 13.33 |

These results show a definite hangfire tendency at low temperatures.

#### Example B

Four parts by weight of a double base powder similar to Example A was blended with one part by weight of a single base powder having substantially the same granulation and specific gravity and was fired at -43.6° F. with a 23.3 grain charge.

| Temp.     | Pressure |        |        | Barrel time, sec./1,000 |      |      |
|-----------|----------|--------|--------|-------------------------|------|------|
|           | Min.     | Mean   | Max.   | Min.                    | Mean | Max. |
| -43.6° F. | 20,900   | 31,700 | 33,700 | 1.90                    | 2.00 | 2.24 |

These results show that the addition of single base smokeless grains prevents excessive barrel time.

#### Example B1

A duplicate of Example B was carried out with a similar but different lot of double base smokeless powder. The results parallel those of Example B and were as follows:

| Temp.     | Pressure |        |        | Barrel time, sec./1,000 |      |      |
|-----------|----------|--------|--------|-------------------------|------|------|
|           | Min.     | Mean   | Max.   | Min.                    | Mean | Max. |
| -45.4° F. | 28,800   | 32,700 | 36,700 | 1.70                    | 2.02 | 2.26 |

#### Example C

A double base powder containing 20% nitroglycerin and coated with 1.5% rosin and 1.5% Ketonone E was tested at a low temperature. This powder did not give excessive pressures at the low temperatures but gave hangfires in the

.25/35 W. C. F. rifle using a 20.0 grain charge. The results are as follows:

| Temp.     | Pressure |        |        | Barrel time, sec./1,000 |      |      |
|-----------|----------|--------|--------|-------------------------|------|------|
|           | Min.     | Mean   | Max.   | Min.                    | Mean | Max. |
| -52.6° F. | 28,800   | 31,800 | 35,000 | 2.27                    | 4.64 | 9.67 |

10

#### Example D

To the powder of Example C was added 25% of a single base powder and the admixture tested in the .25/35 W. C. F. rifle using a 22.0 grain charge. The results were as follows:

| Temp.     | Pressure |        |        | Barrel time, sec./1,000 |      |      |
|-----------|----------|--------|--------|-------------------------|------|------|
|           | Min.     | Mean   | Max.   | Min.                    | Mean | Max. |
| -52.6° F. | 34,100   | 36,500 | 40,000 | 2.53                    | 3.16 | 5.27 |

#### COMPARISON II

In Comparison I powders were tested in the .25/35 W. C. F. rifle. In this comparison similar tests were made in the .30.06 Springfield to show the reduction of hangfires by using the powder admixtures of this invention.

#### Example E

A double base powder containing 20% nitro-glycerin and granulated .045 x .015 x .091 was coated with 1% rosin, 1% butylacetyl ricinoleate and 2% Ketonone E when fired at low temperatures did not develop excessive pressures but hangfires were encountered. The results obtained with a 53.0 grain charge were:

| Temp.     | Pressure |        |        | Barrel time, sec./1,000 |      |      |
|-----------|----------|--------|--------|-------------------------|------|------|
|           | Min.     | Mean   | Max.   | Min.                    | Mean | Max. |
| 73° F.    | 52,200   | 53,000 | 55,000 | 2.76                    | 2.85 | 3.00 |
| -50.5° F. | 41,100   | 43,600 | 47,000 | 2.74                    | 3.38 | 7.45 |

#### Example F

To the powder of Example E was added 15% single base powder. When the admixture was fired using a 49.6 grain charge, the results were:

| Temp.     | Pressure |        |        | Barrel time, sec./1,000 |      |      |
|-----------|----------|--------|--------|-------------------------|------|------|
|           | Min.     | Mean   | Max.   | Min.                    | Mean | Max. |
| 72° F.    | 45,500   | 47,700 | 49,300 | 2.00                    | 2.15 | 2.34 |
| -50.5° F. | 37,500   | 39,700 | 43,500 | 2.16                    | 2.64 | 4.00 |

A blend using 25% single base powder gave similar results.

#### COMPARISON III

In this comparison is shown the excessive pressures obtained when double base powders are shot at low temperatures and the normal pressures obtained when single base powders are admixed therewith.

#### Example G

A double base powder containing 20% nitro-glycerin, granulated .045 x .015 x .091 and coated with 1.25% rosin and 1.25% dinitrotoluene was

fired in a .25/35 W. C. F. rifle at 78° F. and -49° F. using a 23 grain charge. The results were:

| Temp.   | Pressure |        |        |
|---------|----------|--------|--------|
|         | Min.     | Mean   | Max.   |
| 78° F.  | 31,100   | 31,900 | 33,200 |
| -49° F. | 31,100   | 33,200 | 50,000 |

#### Example H

To the powder of Example G was added 20% single base powder having approximately the same granulation and the admixture was fired in the .25/35 W. C. F. rifle at 82° F. and -49° F. using a 22.8 grain charge. The results were:

| Temp.   | Pressure |        |        |
|---------|----------|--------|--------|
|         | Min.     | Mean   | Max.   |
| 82° F.  | 30,800   | 31,100 | 31,600 |
| -49° F. | 31,100   | 33,000 | 40,600 |

#### Example I

A double base powder containing 20% nitro-glycerin, granulated .045 x .015 x .091 and coated with 1.5% rosin and 1% dinitrotoluene was fired in the .25/35 W. C. F. rifle at 76° C. and -47.2° F. using a 23.5 grain charge. The results were:

| Temp.     | Pressure |        |        |
|-----------|----------|--------|--------|
|           | Min.     | Mean   | Max.   |
| 76° F.    | 30,900   | 31,600 | 32,200 |
| -47.2° F. | 34,700   | 45,600 | 51,000 |

#### Example J

To the powder of Example I was added 20% single base powder having approximately the same granulation and the admixture was fired in the .25/35 W. C. F. rifle at 78° F. and -45.4° F. using a 23.7 grain charge. The results were:

| Temp.     | Pressure |        |        |
|-----------|----------|--------|--------|
|           | Min.     | Mean   | Max.   |
| 78° F.    | 31,700   | 33,100 | 34,000 |
| -45.4° F. | 35,600   | 38,600 | 42,000 |

The above blends gave satisfactory ballistics at low temperatures while the double base powder grains alone when fired at low temperatures showed excessive pressures.

In the above examples, the results are an average of ten rounds, except in Examples B, F and H. In these examples, five rounds were fired. Further, in the above examples in which the .25/35 W. C. F. rifle was used, all bullets were Winchester 117 grain S. P. bullets except those in Examples C and D which used Remington 117 grain Express mushroom bullets. The bullets used in the .30-06 Springfield rifle were F. A. 173 grain 9° B. T. bullets. Also, in the above examples, all pressure results are expressed in pounds per square inch.

In the above examples, most results have been obtained in the .25/35 W. C. F. rifle but these improvements are also obtained in the various known rifles such as the .30-06 Springfield, .303 British, .30 W. C. F. and other such rifles.

From the above examples, the advantages of

using powder in accordance with this invention are shown to be the prevention of excessively high breech pressures at sub-zero temperatures and the elimination of hangfires during operation of rifles at sub-zero temperatures. These two items are most advantageous when the rifle is used in aerial warfare, as in most aerial warfare the temperature is quite low. However, many other occasions arise where rifles are operated in sub-zero temperatures and this invention therefore finds many applications.

What I claim and desire to protect by Letters Patent is:

1. A propellant powder charge including an admixture of double base smokeless powder surface modified and characterized by producing breech pressures when fired at sub-zero temperatures which are not substantially greater than those produced when fired at ordinary temperatures, and a single base propellant powder in an amount from about 10 to about 30% by weight, sufficient to allow ready ignition, whereby ignition and firing characteristics are obtained which prevent hangfires at sub-zero temperatures.

2. A propellant powder charge comprising coated double base grains and uncoated single base grains of substantially the same granulation and specific gravity, said powder charge characterized by an ability of expelling a bullet from a rifle in substantially the same length of time at sub-zero temperatures as is required for expelling said bullet at normal temperatures said single base grains being present in amount from about 10 to about 30% by weight.

3. A propellant powder charge comprising an admixture of coated double base powder grains and single base grains, said grains being of substantially the same granulation and specific gravity, and the said double base grains coated with an admixture of an alkyl ester of a higher fatty acid and a non-volatile solvent for the said nitrocellulose said single base grains being present in amount from about 10 to about 30% by weight.

4. A propellant powder adapted for use at sub-zero temperatures, which powder comprises an

10 5 admixture of double base coated grains and single base uncoated grains, said grains having approximately the same granulation and specific gravity, the double base grains coated with an admixture of non-volatile, non-explosive organic deterrent material which is a non-solvent for the nitrocellulose but compatible therewith, and a non-volatile solvent for said nitrocellulose, whereby a propellant powder is produced which expels a bullet from a barrel in approximately the same length of time at sub-zero temperatures as at normal temperatures said single base grains being present in amount from about 10 to about 30% by weight.

15 5. A propellant powder adapted for use at sub-zero temperatures which comprises a blend of grains of double base progressive-burning smokeless powder, characterized by an ability to maintain normal breech pressures when fired at sub-zero temperatures and a single base progressive-burning smokeless powder characterized by a granulation density substantially equivalent to the granulation and density of the said double base powder, said blend including sufficient single base powder grains to effect easy ignition and said blend characterized by an ability to expel a bullet from a barrel at sub-zero temperatures in substantially the same length of time required to expel said bullet at normal temperatures said single base grains being present in amount from about 10 to about 30% by weight.

20 6. An improved propellant powder comprising an intimate admixture of double base and single base smokeless powder grains, said double base powder being surface modified with an admixture of a non-volatile, non-explosive organic deterrent material which is a non-solvent for the nitrocellulose but compatible therewith, and a non-volatile solvent of said nitrocellulose, said single base powder present in an amount from about 10 to about 30% by weight, sufficient to characterize the admixture as being of normal ignition and burning properties when fired at sub-zero temperatures.

ELTON R. ALLISON.